

2,947,621

## TERNARY ALLOYS OF URANIUM, COLUMBIUM, AND ZIRCONIUM

Frank G. Foote, Chicago, Ill., assignor to the United States of America as represented by the United States Atomic Energy Commission

No Drawing. Filed Sept. 13, 1948, Ser. No. 49,128

12 Claims. (Cl. 75—122.7)

This invention relates to ternary alloys and particularly to ternary alloys of uranium useful as neutron-reflecting materials in a fast neutron pile, which alloys are especially resistant to corrosion caused by oxidative processes of aqueous or gaseous origin.

During the course of the investigation of the problem of the susceptibility of uranium metal to oxidative corrosion, it has been discovered that uranium metal in the gamma phase has greater resistance to corrosion by oxidation.

It is therefore an object of this invention to provide compositions of uranium which are resistant to corrosion, and particularly compositions of uranium wherein at least a portion of said uranium is in the corrosion resistant gamma phase.

It is a further object of this invention to provide materials for use in neutronic reactors which necessarily consist predominantly of uranium metal and have the necessary characteristics with respect to neutron capture cross-sections. This object is attained most satisfactorily by alloying uranium metal with materials which will impart the desired corrosion resistance to the uranium metal without adversely affecting the nuclear characteristics of the uranium metal.

It is thus a further object of this invention to provide compositions of uranium having a minimum total alloy content and yet attain maximum resistance to corrosion in said uranium materials.

A still further object of this invention is to provide a process for the preparation of the above-mentioned materials which have the desired physical and nuclear properties.

Further objects and advantages of this invention will be apparent from further examination of the specification.

In accordance with the subject matter of this invention it has been discovered that uranium metal becomes stabilized in the gamma phase when closely alloyed with minor amounts of columbium and zirconium.

Such alloys, which are predominantly uranium having columbium and zirconium as minor alloying materials, have been found to possess properties superior to those found in binary alloys of uranium wherein the uranium metal is alloyed with either columbium or zirconium alone. In order to stabilize uranium metal in the non-corrodible gamma phase, only small percentages of these minor alloy materials, preferably at least about two percent by weight, have been found to be effective. In fact, the ternary alloys which are predominantly uranium and contain a minimum of about two percent by weight of total alloy material, namely, zirconium and columbium, have been found to be superior to those binary alloys of uranium and zirconium or uranium and columbium having an equal or greater total content of alloy material.

From among those ternary alloys of uranium having a minimum total alloy content of columbium and zirconium, those having a total alloy content wherein the ratio

of columbium to zirconium is at least approximately 2 to 1 are preferred since they show greater resistance to corrosion. A total alloy content ranging from two percent to eight percent by weight is suitable for most purposes, however, the alloy consisting predominantly of uranium metal alloyed with as little as two percent by total weight of the alloying materials columbium and zirconium wherein the ratio of columbium to zirconium is approximately 2 to 1 is superior with respect to corrosion resistance to those containing a greater total alloy content.

Throughout this specification, by the term "resistance to corrosion" is meant that an alloy can withstand temperatures between 150 and 200° C. during exposure either 15 to boiling water or to air at a speed of about 150 feet per second. In practice most of these alloys will be subjected to conditions such that the temperature and air speed would not usually exceed 100° C. and 150 feet per second, respectively, and for this purpose I have 20 found that an alloy may be deemed satisfactory when the corrosion rate after 500 hours in test is not in excess of .01 mg./cm.<sup>2</sup>/hr.

As noted before, I have found that uranium metal cast in the high temperature gamma phase shows greater 25 resistance to corrosion than in any other phase. While I do not wish to be bound by any theory as to the mechanism of corrosion, it is perhaps worthy of note that corrosion of uranium metal is attributed to the transformation of uranium metal in the gamma phase to 30 a less corrosion-resistant phase. It is also possible that the gamma phase becomes progressively less corrosion-resistant directly with an increase in temperature, particularly at temperatures in excess of 200° C. It appears, therefore, that the addition to uranium of between two 35 and eight percent by weight of the minor alloying elements, columbium and zirconium, serves to stabilize the uranium metal in the corrosion-resistant gamma phase either by retarding the inception of corrosion, that is, by extending the threshold level or time necessary for the 40 metal to be affected by oxidation; or, after the threshold has been attained, by reducing the rate of oxidation which has begun. It has been noted that columbium is more effective than zirconium in imparting to uranium metal a greater threshold value and also reducing the rate of 45 oxidation once this threshold has been attained.

In accordance with this invention, the process for preparing the ternary alloys comprising the subject matter of this invention comprises casting uranium metal at an elevated temperature, suitably at about 1000° C., with 50 the desired total weight percent of minor alloy materials, namely, columbium and zirconium. The metallic mixture formed thereby contains uranium metal, at least a portion of which is in the gamma phase on account of the elevated casting temperature, with the minor alloying 55 constituents in solid solution of uranium in the as-cast form. In order to homogenize this metallic solution mixture, the alloy mixture is subjected to a solution heat treatment consisting of an extended heating at a temperature of about 1000° C. for a period ranging from about 60 300 hours to 768 hours. The homogeneous mixture of metals is then either quenched immediately or first soaked at a temperature of 850° C. which is then followed by either rapid or slow quenching. However, it has been noted that the amount of gamma phase retained in the 65 uranium material is favored considerably by an increase in the quenching rate which is suitably achieved by reducing the cross-sectional area of the metal by any suitable means such as rolling or extrusion, since the rate of quenching, in the metal under treatment, increases 70 directly with the reduction in cross-sectional area. Preservation of uranium metal in the gamma phase by alloying with columbium and zirconium metal is most

certain when the alloys are prepared according to the process set forth herein.

The superiority of the ternary alloys comprising the subject matter of this invention will be apparent from the following descriptions and tables wherein the composition, heat treatment and conditions of test are set forth.

An alloy sample which averaged 0.4 weight percent zirconium and 2.17 weight percent columbium and the balance uranium metal was rolled to a  $\frac{5}{8}$ -inch rod at  $850^{\circ}$  C. Specimens of this sample were subjected to a dynamic air corrosion test for 1300 hours wherein the air speed to which the specimens were subjected was about 100 feet per second and the temperature was  $150^{\circ}$  C. The weight gain rate for seven specimens varied from 0.0006 to 0.0018 mg./cm.<sup>2</sup>/hr. The average weight gain of 0.0014 mg./cm.<sup>2</sup>/hr. was attained after 500 hours. The alloy was then treated with 30% nitric acid to remove any oxide formed during the test and the resultant weight loss was plotted against time to obtain a value for the total weight of uranium converted to oxide. These figures showed the average rate of uranium metal oxidized was 0.008 mg./cm.<sup>2</sup>/hr. which indicates that the range of weight gain quoted above is equivalent to 0.0035 to 0.010 mg./cm.<sup>2</sup>/hr. as an average rate of oxidation of metal from metal surfaces.

In a further investigation of the uranium-columbium-zirconium system, specimens of binary uranium-columbium and uranium-zirconium alloys were homogenized for one week at  $1000^{\circ}$  C. then soaked at  $850^{\circ}$  C. followed by a fast brine quench. The samples were ground on #250 grit emery paper, the total surface areas measured and initial weights noted. Each sample was placed in a water glass to collect all the oxide formed and samples were then placed in an oven at  $150^{\circ}$  C. with slow air circulation. Results of this test are shown by the following data obtained for the five most active specimens.

| Nominal wt. percent alloy | Hours in Test in air at $150^{\circ}$ C. | Wt. change, mg./cm. <sup>2</sup> /hr. | Remarks                                   |
|---------------------------|------------------------------------------|---------------------------------------|-------------------------------------------|
| (pure U)-----             | 282                                      | 0.64                                  | Fairly constant rate gain.                |
| 0.3% Cb-----              | 282                                      | 0.26                                  | Do.                                       |
| 0.55% Cb-----             | 282                                      | 0.25                                  | Threshold reached corrosion after 50 hrs. |
| 0.9% Cb-----              | 282                                      | not detd.                             | Threshold after 120 hrs.                  |
| 1.0% Zr-----              | 282                                      | 0.17                                  | Fairly constant rate gain.                |
| 2.0% Zr-----              | 282                                      | 0.048                                 | Corrosion threshold reached after 50 hrs. |
| 3.4,6% Zr-----            | 282                                      | not detd.                             | Threshold reached at 120 hrs.             |

The procedure for the previous test was repeated using

TABLE II

| Percent by wt. Alloy Material (Remaining Percent Uranium) | Heat Treatment |                                            | Time in Test, Hrs. | Wt. Change, Mg./cm. <sup>2</sup> /hr. | Remarks                                                                                                                                      |
|-----------------------------------------------------------|----------------|--------------------------------------------|--------------------|---------------------------------------|----------------------------------------------------------------------------------------------------------------------------------------------|
| Nominal                                                   | Actual         |                                            |                    |                                       |                                                                                                                                              |
| Pure Uranium*-----                                        |                | Slag Metal (As-cast)-----                  | 110                | 2.3                                   | Fairly consistent rate.                                                                                                                      |
| Do*-----                                                  |                | Slow-cooled and Worked-----                | 310                | .77                                   | Work sample corroded faster at first.                                                                                                        |
| Do*-----                                                  |                | Slow-cooled and Unworked-----              | 310                | .77                                   | A fast corrosion rate at beginning of test.                                                                                                  |
| 2 Cb*-----                                                | 2.1 Cb         | As-cast Furnace-cooled-----                | 540                | .29                                   | Inconsistent rate.                                                                                                                           |
| 4 Cb*-----                                                | 4.6 Cb         | do-----                                    | 562                | .17                                   | Insignificant wt. change first 230 hrs.                                                                                                      |
| 4 Cb-----                                                 | 4.6 Cb         | H.T., 5.5 days at $1,000^{\circ}$ C., W.Q. | 1,708              | -.001                                 | Most wt. change first 200 hrs.                                                                                                               |
| 9 Cb*-----                                                | 10.2 Cb        | As-cast Furnace-cooled-----                | 1,081              | -.0007                                |                                                                                                                                              |
| 9 Cb-----                                                 | 10.4 Cb        | H.T., 11 days at $1,000^{\circ}$ C., W.Q.  | 1,708              | +.0005                                | Most wt. change first 200 hrs.                                                                                                               |
| 20 Cb*-----                                               | 24.8 Cb        | As-cast Furnace-cooled-----                | 560                | none                                  |                                                                                                                                              |
| 20 Cb-----                                                | 23.2 Cb        | H.T., 11 days at $1,000^{\circ}$ C., W.Q.  | 1,708              | none                                  |                                                                                                                                              |
| 2 Zr*-----                                                | 1.9 Zr         | As-cast-----                               | 264                | -.53                                  | Consistent rate.                                                                                                                             |
| 2 Zr-----                                                 | 1.9 Zr         | H.T., 18 hrs. at $850^{\circ}$ C., W.Q.    | 849                | -.41                                  | Fairly consistent rate.                                                                                                                      |
| 2 Zr-----                                                 | 1.9 Zr         | H.T., 53 hrs. at $1,000^{\circ}$ C., W.Q.  | 130                | -.71                                  | Sample fell apart.                                                                                                                           |
| 4.1 Zr*-----                                              | 4.3 Zr         | As-cast-----                               | 398                | -.02                                  | Corroded slowly first 150 hrs.                                                                                                               |
| 4.1 Zr*-----                                              | 4.3 Zr         | H.T., 18 hrs. at $850^{\circ}$ C., W.Q.    | 994                | -.007                                 | Consistent rate.                                                                                                                             |
| 4.1 Zr*-----                                              | 4.3 Zr         | H.T., 53 hrs. at $1,000^{\circ}$ C., W.Q.  | 919                | -.007                                 | Do.                                                                                                                                          |
| 8 Zr*-----                                                | 8.7 Zr         | As-cast-----                               | 400                | -.65                                  | Do.                                                                                                                                          |
| 8 Zr-----                                                 | 8.7 Zr         | H.T., 18 hrs. at $850^{\circ}$ C., W.Q.    | 991                | -.17                                  | Corroded very slowly first 170 hrs.                                                                                                          |
| 8 Zr-----                                                 | 8.7 Zr         | H.T., 53 hrs. at $1,000^{\circ}$ C., W.Q.  | 848                | -.006                                 | Consistent rate.                                                                                                                             |
| 2 Zr; 2 Cb-----                                           |                | H.T., 100 hrs. at $1,000^{\circ}$ C., W.Q. | 733                | none                                  |                                                                                                                                              |
| 4 Zr; 2 Cb-----                                           |                | do-----                                    | 733                | -.0007                                | No wt. change first 240 hrs.                                                                                                                 |
| 6 Zr; 2 Cb-----                                           |                |                                            | 733                | -.00056                               | No wt. change first 400 hrs. This alloy is the least stable since a faster quenching rate was required to retain completely the gamma phase. |

See footnotes at end of table.

binary and ternary alloy samples which had been in the oven for a total of 785 hours, and the samples were cleaned as before in 30% nitric acid and the weight losses measured. Results of these tests showed that pure uranium begins to oxidize as soon as it is put under test and proceeds at a constant rate corresponding to a loss of about 0.66 mg./cm.<sup>2</sup>/hr., which corrosion rate is considerably reduced by very low alloy additions of columbium, zirconium, or mixtures thereof. Slightly larger additions cause the alloy to remain stable until a threshold is reached and further additions of alloy extend the length of time before the threshold is attained and reduce the oxidation rate thereafter.

The binary uranium alloy containing 0.9% columbium was approximately as good as the 2.5%-zirconium binary uranium alloy, both having thresholds at approximately 50 to 60 hours. The binary uranium-4.2% columbium alloy had a threshold of 180 to 200 hours and thereafter gained weight very slowly. The binary uranium alloy containing 11% columbium and the ternary uranium alloys containing 2% columbium-1% zirconium, and 3% columbium-1% zirconium showed hardly detectable thresholds. The threshold for the alloy of uranium containing 2% columbium-1% zirconium was roughly 300 hours and after a total of 785 hours in test, the alloy had been oxidized at an average rate of 0.005 mg./cm.<sup>2</sup>/hr. at  $150^{\circ}$  C. At the end of the test it was coated with a uniform thin tenacious film. The following tables further illustrate the relative efficiency of different percentages of columbium and zirconium in effecting improvements in the physical properties such as resistance to corrosion and hardness values in uranium metal.

TABLE I

## Rockwell C values of U-Cb-Zr alloys

| Alloy Composition (Nominal wt. % added to U):                                                            | 2  | 2  | 2  | 4  | 4  | 6  |
|----------------------------------------------------------------------------------------------------------|----|----|----|----|----|----|
| Percent Cb-----                                                                                          | 2  | 4  | 6  | 2  | 4  | 2  |
| Percent Zr-----                                                                                          | 2  | 4  | 6  | 2  | 4  | 2  |
| Alloy Treatment:                                                                                         |    |    |    |    |    |    |
| Homogenized 768 hrs. at $1,000^{\circ}$ C. and water quenched-----                                       | 35 | 31 | 32 | 20 | 20 | 90 |
| Homogenized 768 hrs. at $1,000^{\circ}$ C., soaked at $850^{\circ}$ C. for 256 hrs., air-cooled-----     | 53 | 53 | 52 | 30 | 46 | 21 |
| Homogenized at $1,000^{\circ}$ C. for 768 hrs., heated at $600^{\circ}$ C. for 64 hrs., air-cooled-----  | 30 | 30 | 31 | 30 | 30 | 38 |
| Homogenized at $1,000^{\circ}$ C. for 768 hrs., heated at $600^{\circ}$ C. for 256 hrs., air-cooled----- | 35 | 31 | 33 | 30 | 31 | 31 |

TABLE II—Continued

| Percent by wt. Alloy Material<br>(Remaining Percent Uranium) |        | Heat Treatment                        | Time in<br>Test,<br>Hrs. | Wt. Change,<br>Mg./cm. <sup>2</sup> /hr. | Remarks                                         |
|--------------------------------------------------------------|--------|---------------------------------------|--------------------------|------------------------------------------|-------------------------------------------------|
| Nominal                                                      | Actual |                                       |                          |                                          |                                                 |
| 2 Zr; 4 Cb.                                                  |        | H.T., 100 hrs. at 1,000° C., W.Q.     | 733                      | +.00014                                  | +0.2 mg. wt. change.                            |
| 4 Zr; 4 Cb.                                                  |        | do                                    | 733                      | +.0002                                   | Do.                                             |
| 2 Zr; 6 Cb.                                                  |        |                                       | 733                      | none                                     |                                                 |
| 2 Zr; 2 Cb.                                                  |        | H.T., 250 hrs. at 850° C., Air-cooled | 446                      | +.0004                                   | +0.3 mg. wt. change.                            |
| 4 Zr; 2 Cb.                                                  |        | do                                    | 446                      | +.0003                                   | +0.2 mg. wt. change.                            |
| 6 Zr; 2 Cb.                                                  |        | do                                    | 446                      | -.0017                                   | All wt. loss first 260 hrs.                     |
| 2 Zr; 4 Cb.                                                  |        | do                                    | 446                      | +.0006                                   | +0.3 mg. wt. change (consistent increase).      |
| 4 Zr; 4 Cb.                                                  |        | do                                    | 446                      | +.0006                                   | +0.3 mg. wt. change (no change first 260 hrs.). |
| 2 Zr; 6 Cb.                                                  |        | do                                    | 445                      | +.0004                                   | +0.3 mg. wt. change (consistent increase).      |
| 2 Zr; 2 Cb.                                                  |        | H.T., 250 hrs. at 725° C., Air-cooled | 446                      | -.0008                                   | All wt. loss first 90 hrs.                      |
| 4 Zr; 2 Cb.                                                  |        | do                                    | 446                      | +.00016                                  | +0.1 mg. wt. change.                            |
| 6 Zr; 2 Cb.                                                  |        | do                                    | 446                      | -.0005                                   | All wt. loss during first 260 hrs.              |
| 2 Zr; 4 Cb.                                                  |        | do                                    | 446                      | +.0007                                   | +0.4 mg. wt. change.                            |
| 4 Zr; 4 Cb.                                                  |        | do                                    | 445                      | +.0005                                   | Do.                                             |
| 2 Zr; 6 Cb.                                                  |        | do                                    | 445                      | +.0001                                   | +0.1 mg. wt. change.                            |

pH of H<sub>2</sub>O 5.6-5.8. H.T.—High temperature. W.Q.—Water quenched.

NOTE.—In the foregoing tests, the asterisk (\*) indicates that the corrosion product was removed by immersing for two to three minutes in 25% (by wt.) nitric acid solution. The remaining samples listed showed no reaction with nitric acid so no attempt was made to clean them before weighing. All samples were rinsed in distilled water and blown dry.

It will be apparent to those skilled in the art to which this invention pertains that various modifications can be made without departing from the preferred embodiments of this invention as disclosed herein, and thus it is not intended that the subject invention be limited other than by the scope of the appended claims.

What is claimed is:

1. An alloy consisting substantially of uranium, zirconium, and columbium wherein the amount of uranium metal is greater than the total zirconium and columbium content and is the major constituent of the alloy.

2. An alloy consisting substantially of uranium as the predominant metal, zirconium and columbium wherein the total content of said minor alloying elements is between two and eight percent by weight.

3. A ternary alloy consisting substantially of a predominant amount of uranium metal and zirconium and columbium wherein the minor alloying elements columbium and zirconium are each present in amounts between 1 and 4 percent by weight.

4. An alloy consisting essentially of uranium metal, zirconium and between 1 and 4 percent by weight columbium, wherein said columbium is present in excess of the zirconium.

5. An alloy consisting essentially of uranium metal and a total content of columbium and zirconium between two and eight percent wherein said columbium and zirconium are each present in amounts between one and four percent by weight.

6. An alloy consisting essentially of uranium metal and zirconium and columbium as minor alloying elements wherein the total percent of said minor alloying elements is at least about two percent.

7. An alloy consisting essentially of uranium and a total of at least two percent minor alloying materials consisting of columbium and zirconium wherein the ratio of said columbium to zirconium is at least about 2 to 1, respectively.

8. A process for preparing an alloy of uranium comprising casting at a high temperature uranium alloy consisting substantially of uranium as the predominant metal

and a total of at least two percent of minor alloying elements, namely, columbium and zirconium, heat treating said alloy at an elevated temperature to obtain a homogeneous composition and subsequently quenching said homogeneous alloy composition.

9. The process of claim 12 wherein said alloy of uranium is subjected to prolonged heat treatment at a temperature of 1000° C. and subsequently quenched from a temperature of at least 725° C.

10. A process for preparing an alloy of uranium comprising adding the total minor alloying elements, columbium and zirconium, to uranium during the casting of said uranium, heat treating the alloy formed thereby at 1000° C. and quenching said alloy mixture from a temperature of at least 725° C.

11. The process of claim 14 wherein said minor alloying elements are added in the approximate ratio of at least 2 parts columbium to 1 part zirconium in amounts sufficient to bring the total content of minor alloying elements to between two and eight percent by weight.

12. A process for preparing a corrosion-resistant alloy of uranium comprising adding columbium and zirconium, in amounts sufficient to bring the total content of minor alloying elements to between two and eight percent by weight, to uranium metal during the casting of said uranium metal, heat treating at 1000° C. the alloy formed thereby, and quenching said alloy mixture from a temperature of at least 725° C.

#### References Cited in the file of this patent

#### UNITED STATES PATENTS

55 2,237,872 Badger ----- Apr. 8, 1941

#### FOREIGN PATENTS

114,150 Australia ----- May 2, 1940  
561,592 Great Britain ----- May 25, 1944

#### OTHER REFERENCES

60 Journal of the American Chemical Society, vol. 68, pages 2421, 2422 (1946).

UNITED STATES PATENT OFFICE  
CERTIFICATE OF CORRECTION

Patent No. 2,947,621

August 2, 1960

Frank G. Foote

It is hereby certified that error appears in the printed specification of the above numbered patent requiring correction and that the said Letters Patent should read as corrected below.

Column 3, line 34, for "water" read -- watch --; column 6, line 28, for the claim reference numeral "12" read -- 8 --; line 38, for the claim reference numeral "14" read -- 10 --.

Signed and sealed this 25th day of April 1961.

(SEAL)

Attest:

ERNEST W. SWIDER

Attesting Officer

DAVID L. LADD

Commissioner of Patents